

## UNITED STATES PATENT OFFICE

1,956,552

## COATING MOLD

Alexander H. Fosdick, Bethlehem, Pa., assignor  
to Bethlehem Steel Company, a corporation of  
Pennsylvania

No Drawing. Application December 11, 1931,  
Serial No. 580,497

4 Claims. (Cl. 22—192)

My invention relates to a coating for molds in which molten metal is cast.

The main object of my invention is to provide an improved coating for the molds of continuous casting machines by means of which molten blast furnace iron is converted into pigs.

Such casting machines consist essentially of one or more endless chains or belts of trough shaped metal molds which receive molten iron at one end of their flight, carry it through water sprays and discharge it as solidified pig iron at the other end. During their return flight the molds are inverted, that is, their openings face downward and it is common practice to spray them at some point in this portion of their travel with a coating material. The main functions of this coating are: to prevent the pigs sticking to the molds, to prevent excessive chilling of the pigs and to prolong the life of the molds. The usual method of applying the coating is to pass the molds over a tank containing the coating material and to spray the same onto the molds by means of steam ejectors located in the tank.

My improved mold coating is essentially a wa-  
ter suspension of an oily substance and a finely  
divided refractory pigment. As the latter of  
these two constituents I prefer burnt dolomite  
and my preferred practice is to maintain an ex-  
cess of same in the coating tank and to agitate  
the mixture with steam. To the suspension thus  
formed I prefer to add raw coal tar in the ratio  
of one part of tar to four parts of the dolomite  
wash. This forms a light brown mixture in  
which the tar is easily maintained by agitation  
in a finely dispersed condition.

The main function of the oily constituent is to waterproof the deposit formed on the molds by the coating and it will therefore be evident that the proportions of oil and pigment for best results may vary within rather wide limits de-  
pending on the properties of the oil, the average  
temperature of the molds, etc. The novel im-  
provement constituting the basis of my invention  
is the combination in aqueous suspension of a  
pigment with an insoluble heavy oil and I there-  
fore do not wish to be limited to a particular  
pigment or oil or to the proportions thereof set  
forth above. While I prefer burned dolomite as  
the pigment, various other finely divided refrac-  
tory substances such as common lime or fire clay  
may also be successfully used. In place of tar,  
any other heavy oil such as a heavy fraction of  
petroleum may be used. By "heavy oil" I refer  
to oils of high boiling point such as are common-  
ly used alone as mold coatings.

The coatings for pig molds which hitherto have been most widely used are aqueous suspen-  
sions of dolomite, common lime or fire clay.  
Coatings of this kind build up a deposit of soft  
porous material on the surface of the molds  
which normally becomes quite thick—perhaps a  
half inch or more on certain parts of the mold.  
This deposit successfully protects the molds, pre-  
vents the pigs from sticking and protects them  
from excessive chilling. Such coatings, however,  
are subject to a serious disadvantage in that they  
retain a certain amount of moisture unless  
special provisions are made for drying the molds  
between the coating tank and the pouring trough.  
The amount of this moisture—or rather the rate  
at which it is evolved is generally insufficient to  
cause explosions or serious spattering of the  
molten iron; but it is sufficient to cause a slow  
boiling action in the metal for some time after it  
is cast. The result of this action is an oxidation  
of certain constituents of the iron and a porous  
condition of the finished pig. This oxidation and  
porosity is not only undesirable from a metal-  
lurgical standpoint but it adversely effects the  
appearance of the product and reduces its sales  
appeal. It has also been stated in various U. S.  
patents that basic materials which adhere to  
pig iron cast in such coatings are detrimental to  
cupola melting practice.

To overcome these defects it has been proposed  
to substitute tar or other heavy oils for the lime  
or clay wash. Although the use of tar eliminates  
the oxidizing effects above referred to it has been  
found that it does not prevent pigs sticking to  
the molds. It also produces an objectionable  
amount of smoke and flame when it comes in  
contact with molten iron. For these and other  
reasons it has never been widely adopted as a  
coating for pig molds.

The failure of tar to prevent sticking is readily  
explainable if we bear in mind that pig molds  
inevitably become distorted and roughened in  
service so that they contain reentrant crevices  
and pockets. A coating to be satisfactory should  
therefore build up a deposit of sufficient thick-  
ness to fill out these surface inequalities. My  
improved coating builds up a deposit almost if  
not quite as thick as the plain pigment coating  
which at the same time retains so little water  
that boiling of the molten iron is avoided. Ex-  
amination of the deposit produced by my coat-  
ing shows that the tar is burned out of the sur-  
face layer only and that a considerable part of  
it is driven into and absorbed by the underlying  
mass—thereby filling the pores of same and pre-  
110

venting the absorption of water. When molten iron is poured into molds coated with my coating there is practically no smoke or flame and boiling of the metal ceases in a few seconds. Thereafter 5 the metal lies as quietly as in tarred molds.

Having thus described my invention what I claim as new and desire to secure by Letters Patent is:

1. The process of coating pig casting molds 10 which consists in repeatedly applying thereto a wash consisting of an aqueous suspension of a refractory pigment and a heavy oil and in casting pigs in said molds between successive applications of said wash.

15 2. The process of coating pig casting molds which consists in repeatedly applying thereto a wash consisting of an aqueous suspension of

burned dolomite and a heavy oil and in casting pigs in said molds between successive applications of said wash.

3. The process of coating pig casting molds 80 which consists in repeatedly applying thereto a wash consisting of an aqueous suspension of burned dolomite and tar and in casting pigs in said molds between successive applications of said wash.

4. The process of coating pig casting molds 85 which consists in repeatedly applying thereto a mixture containing about 80% of an aqueous suspension of burned dolomite and about 20% of tar and in casting pigs in said molds between successive applications of said mixture. 90

ALEXANDER H. FOSDICK.

20 95

25 100

30 105

35 110

40 115

45 120

50 125

55 130

60 135

65 140

70 145

75 150